

## UNITED STATES PATENT OFFICE

2,344,629

## REMOVAL OF ZINC FROM LEAD

Walter T. Monson, Newark, N. J., assignor to The American Metal Company, Limited, New York, N. Y., a corporation of New York

No Drawing. Application February 11, 1942,  
Serial No. 430,362

4 Claims. (Cl. 75—78)

This invention relates to the removal of zinc from lead, especially lead which has been desilverized and contains only a small percentage of other impurities than zinc.

In the usual of refining lead to produce desilverized lead, one step consists of removing silver by treating with zinc. The silver is removed with most of the zinc as a zinc crust. However, .5 to .6% of zinc remains dissolved in the lead and this must be removed to make a fully refined lead. Formerly this zinc was removed by pumping the lead into a refining furnace and blowing steam into the metal, whereby a zinc-oxide-lead-oxide slag was formed and skimmed off. More recently zinc has been removed by treating the lead in a kettle with calcium-hydroxide, sodium-hydroxide or similar chemical and stirring in order to form a dross containing the zinc. In another process zinc has been removed by passing chlorine into the impure lead and forming zinc chloride which was skimmed from the metal bath. All these methods have required expensive reagents and the cost of removal has been appreciable.

An important object of my invention, accordingly, is to produce a simple and efficient process for the removal of zinc from desilverized lead at relatively low cost.

The invention accordingly consists of a process comprising treating impure lead containing zinc but substantially free from other impurities by stirring the lead in molten condition at a relatively high speed while maintaining it at a temperature of about 1100—1200° F. in the absence of an alkali-metal oxidizing agent, with an oxidizing agent selected from the group consisting of air and added powdered litharge, and added powdered litharge alone, where air and litharge are used as the oxidizing agent, the litharge being added substantially at the commencement of the stirring operation and constituting a quantity in addition to that formed by contact of the air with the impure lead; and the stirring being conducted under an atmosphere of inert gas when litharge alone is used as the oxidizing agent. A dross is formed thereby consisting substantially of zinc oxide and lead oxide. I prefer to add the litharge as a slag containing zinc oxide in addition to the litharge or lead oxide.

I have found in accordance with my invention that by stirring the lead-zinc bath at high-speed and high-temperature with oxidation, I can quickly remove all but traces of zinc from metal containing .5 to .6% or more of zinc and

produce a dross that contains 25% or more zinc content. The basis of my dezincing process is the selective oxidation of the zinc in the desilverized lead bath and the additional concentration by replacement reactions between lead oxide in the dross and zinc in the lead. The typical replacement reaction is:



(Lead oxide plus zinc) (Zinc oxide plus lead)

10 I have operated the process of my invention at speeds of about 900 R. P. M. and above and temperatures of 950° F. and above, with apparatus similar to that described by Harper and Reinberg in U. S. Patent No. 2,155,545 with excellent results. However, in my preferred practice, the temperature is kept over 1100° F. and the stirring speed about 1700 R. P. M. This gives a higher rate of zinc removal and a higher grade dross.

20 In practising my invention, I prefer to place an oxide cover of zinc-oxide-lead-oxide slag on the bath substantially at the commencement of the operation but litharge as such may be employed if desired. The use of a starting oxide makes it possible to produce a high grade dross with a fast rate of removal.

When dezincing, the dross is almost always wet at the start, even if a dry dross is added as 30 starting oxide. In order to get efficient dezincing, it has been found desirable to add a little rosin and sal ammoniac (ammonium chloride) after which the dross stays dry until dezincing is complete. A cover over the kettle 35 has been found helpful when working with dry drosses to keep dust from passing out into the atmosphere, but the cover is sufficiently loose to permit entry of air to permit oxidation of further quantities of lead used up in the above replacement reaction.

Desilverized lead contains very small amounts of impurities other than zinc, so that the only two metals available for oxidation are zinc and lead. It is known that litharge formation is 45 very rapid under oxidizing conditions when the impurity content of the lead is low. Therefore, as soon as the first portions of zinc with the small amounts of impurities present have been oxidized into the dross, the formation of litharge becomes rapid and has a tendency to dilute the zinc oxide formed. Hence the first drosses are higher in zinc, whereas the later drosses start in to decrease in zinc content and go up in lead content. I have found that if the dross is skimmed after two or more alternate

intervals of stirring and skimming, the last dross skimmed may be used on the next charge to be treated for zinc removal with very good results.

I have also found that it is possible with my process to make drosses very high in zinc and low in lead, by stirring a zinc-oxide-lead-oxide dross on a bath of zinc, or metal bath high in zinc content. The dross stirred in may be of the type produced by my process described above, or it may be from some other source. By stirring in at high speed and high temperature a dross containing, say, from around 10 to 30% zinc as oxide and the balance lead as oxide, it has been possible to bring the zinc content up to over 70%.

In employing metallic baths which are high in zinc in order to make a dross with a high zinc-content, I have found that too much oxidation of the zinc bath occurs by air drawn in at the vortex caused by the impeller unless precautions are taken to prevent it. The air thus drawn in acts to convert the zinc in the bath to zinc oxide in excess of that which should be formed by replacement reactions with lead oxide. In this operation, it is desirable to get as much replacement reaction between lead oxide in the dross and metallic zinc as possible in order to obtain the greatest economic advantages of the invention. I have accordingly overcome the above-mentioned difficulty by operating in a neutral atmosphere to prevent primary oxidation of the zinc. In order to do this, I seal the kettle with a gas-tight cover having an inlet for a neutral gas and an outlet. A snug-fitting sleeve for the shaft from the motor to the impeller decreases the amount of gas used since the neutral atmosphere on the bath is kept under a slight pressure in order to insure that no air enters. In my preferred practice, I have found nitrogen or carbon dioxide ( $CO_2$ ) to be very efficient for this purpose, but other gases which would retard or prevent the formation of zinc oxide due to atmospheric conditions over the metal bath may also be used.

In order to better illustrate my process, the following examples are given but the invention is not to be considered as limited thereto except as indicated in the appended claims.

#### Example 1

In an apparatus such as that shown in Patent No. 2,155,545, to 7,600 lbs. of lead bullion containing .776% zinc, the balance being substantially all lead, was added 595 lbs. of oxide from another kettle assaying 20.45% zinc as oxide and the balance lead as oxide. The bath was stirred with access of air for one hour at a speed of 1050 R. P. M. and 1100° F. The lead at the end of the hour contained only a trace of zinc. The dross skimmed off assayed 25.27% Zn.

The metal balance and rate of removal were as follows:

|                                        |               |
|----------------------------------------|---------------|
| 7,600 lbs. bullion containing          |               |
| .776% Zn                               | lbs. Zn 59    |
| 595 lbs. oxide containing              |               |
| 20.45% Zn                              | do 121.7      |
| Total input                            | do 180.7      |
| 773 lbs. zinc oxide skimmed containing |               |
| 25.27% Zn                              | lbs. Zn 195.3 |
| Rate of zinc removed                   |               |
| lbs. per hour per ton                  | 15.5          |

#### Example 2

The following example illustrates the method used to increase the zinc content of drosses by stirring a lead-oxide-zinc-oxide dross on a bath of zinc or metal high in zinc employing an apparatus as in Example 1. No attempt was made to exclude air from the zinc bath as was done in Example 3 given below. As a result, the amount of zinc entering the dross for each pound of lead reduced is higher in the present example than in Example 3, as indicated by the details of the runs given in the examples.

To 4,640 lbs. of zinc assaying 98.2% Zn and 1.8% Pb, melted in a kettle, was added 335 lbs. of mixed zinc and lead oxide containing 17.99% zinc and 69.6% lead. The bath while open to the air was stirred for 15 minutes at a speed of 1700 R. P. M. and a temperature of 1140° F. The dross skimmed off at the end of the run assayed 69.79% Zn and only 11.8% lead.

Details of the run follow:

| Metal basis | Weight | Per cent Zn | Per cent Pb | Pounds Zn | Pounds Pb |
|-------------|--------|-------------|-------------|-----------|-----------|
| Metal start | 4,640  | 98.20       | 1.8         | 4556.5    | 83.5      |
| Metal end   | 4,515  | 94.20       | 5.8         | 4253.1    | 261.9     |
| Difference  | 135    | -----       | -----       | -303.4    | +178.4    |

For each pound of lead reduced to metal, 1.6 lbs. of zinc were transferred to the dross which is more than the theoretical amount of about .3 lb. This is partly due to zinc entrained in the dross and partly due to primary oxidation by air stirred into the bath.

#### Example 3

In order to prevent the primary oxidation of zinc, during the grading up of zinc drosses, an apparatus like that in Patent No. 2,155,545 was employed but the kettle was covered and a neutral atmosphere was kept over the bath.

In the following example an atmosphere of  $CO_2$  was kept on the bath during the stirring operations. The pressure of the  $CO_2$  gas was maintained at one inch of water above atmosphere pressure to prevent any air from entering.

To 4,996 lbs. of zinc assaying 98.8% Zn and 1.2% Pb was added 286 lbs. of zinc-oxide-lead-oxide dross running 29.07% Zn and 57.60% Pb.

The charge was stirred for 30 minutes under an atmosphere of  $CO_2$ , except for the last two minutes when 1 lb. of ammonium chloride ( $NH_4Cl$ ) and 2 lbs. of rosin were added to dry the wet zinc dross.

A temperature of 1160 to 1200° F. was maintained and a stirring speed of 1700 R. P. M.

At the end of the stirring period 316 lbs. of dross were skimmed containing 70.89% Zn and 13.00% Pb.

The details of the run are as follows:

| Metal basis | Weight | Per cent Zn | Per cent Pb | Pounds Zn | Pounds Pb |
|-------------|--------|-------------|-------------|-----------|-----------|
| Metal start | 4,996  | 98.8        | 1.2         | 4,936.0   | 59.9      |
| Metal end   | 4,996  | 96.3        | 3.7         | 4,781.3   | 183.7     |
|             | 31     | -----       | -----       | -154.7    | +123.8    |

In this case, 1.1 lbs. of zinc entered the dross for each pound of lead reduced. In Example 2, 1.6 lbs. of zinc entered the dross for each pound of lead reduced, showing the improvement with

the protective atmosphere in the above Example 3.

A 9½ inch impeller is used in a 40-ton kettle. For a smaller sized kettle, such as a 40-inch kettle, an impeller of 6½ inches may be used. For larger or smaller sized kettles, a variation in the size of the impeller is preferably made, the variation being made in accordance with the dimensions of kettles and impellers mentioned above.

The examples illustrate the invention as I now prefer to practise it, and represent a simple efficient process for treating zinc and lead to form drosses of zinc oxide and lead oxide. These drosses may be further treated to recover the metal values.

Although I have mentioned rosin and ammonium chloride as materials which are preferably employed for drying the dross, other materials may be used instead, such as oil, grease, sawdust, or powdered coal.

What I claim is:

1. A process for treating impure lead containing zinc but substantially free from other impurities which comprises stirring the impure lead in molten condition at high speed while maintaining it at a temperature of about 1100-1200° F. in the absence of an alkali-metal oxidizing agent, with an oxidizing agent selected from the group consisting of air and added powdered litharge, and added powdered litharge alone; where air and litharge are used as the oxidizing agent, the litharge being added substantially at the commencement of the stirring operation and constituting a quantity in addition to that formed by contact of the air with the impure lead; and the stirring being con-

ducted under an atmosphere of inert gas when litharge alone is used as the oxidizing agent; thereby forming a dross consisting substantially of zinc oxide and lead oxide.

5 2. A process for treating an impure lead containing small quantities of zinc but substantially free from other impurities which comprises stirring the impure lead with an oxidizing agent consisting of added powdered litharge and air at 10 about 1100-1200° F. in the absence of an alkali-metal oxidizing agent, the litharge being added substantially at the commencement of the stirring operation and constituting a quantity in addition to that formed by contact of the air with 15 the impure lead, and thereby increasing the zinc oxide content of the dross so that it contains at least 25% zinc as oxide.

3. A process for treating an impure lead containing small quantities of zinc but substantially 20 free from other impurities which comprises stirring the impure lead with an oxidizing agent consisting of added powdered litharge at about 1100-1200° F. in the absence of an alkali-metal oxidizing agent, the stirring being conducted 25 under an atmosphere of inert gas, thereby increasing the zinc oxide content of the dross so that it contains at least 25% zinc as oxide.

4. A process for treating a mixture of zinc and lead which comprises placing a layer of 30 dross consisting of zinc oxide and lead oxide on a bath of zinc and lead in which bath there is a relatively small proportion of lead and stirring the bath and dross layer at about 1100-1200° F. while maintaining an inert atmosphere 35 above the surface of the bath and dross layer, thereby increasing the content of zinc oxide in

WALTER T. MONSON.

CERTIFICATE OF CORRECTION.

Patent No. 2,344,629.

March 21, 1944.

WALTER T. MONSON.

It is hereby certified that error appears in the printed specification of the above numbered patent requiring correction as follows: Page 3, first column, line 5, for "kettle" read --kettle--; and second column, line 36, claim 4, after "in" insert --the dross layer.--; and that the said Letters Patent should be read with this correction therein that the same may conform to the record of the case in the Patent Office.

Signed and sealed this 16th day of May, A. D. 1944.

Leslie Frazer

(Seal)

Acting Commissioner of Patents.